

C. F. SÖDERVALL & H. HELIN.  
METHOD FOR PRODUCING POROUS MATERIALS.  
APPLICATION FILED AUG. 2, 1912.

**1,235,071**

Patented July 31, 1917.



INVENTORS  
Carl Fredrik Södervall  
Henning Helin

BY

*Wm. Greene M. M. & Co.*  
ATTORNEY

# UNITED STATES PATENT OFFICE.

CARL FREDRIK SÖDERVALL, OF KILSMO, AND HENNING HELIN, OF SKÄRBLACKA,  
SWEDEN.

## METHOD FOR PRODUCING POROUS MATERIALS.

1,235,071.

Specification of Letters Patent. Patented July 31, 1917.

Application filed August 2, 1912. Serial No. 712,877.

*To all whom it may concern:*

Be it known that we, CARL FREDRIK Södervall, Brefvens Bruk, Kilsma, Sweden, and HENNING HELIN, Skärblacka, Sweden, subjects of the King of Sweden, have invented certain new and useful Improvements in Methods for Producing Porous Materials, of which the following is a specification.

The present invention relates to a method for producing a material for the working parts of breaking-engines, wood-pulp mills and similar apparatuses intended for grinding wood-pulp and the like. Such working parts must have a porous and crystalline structure, so that they will be very durable and also act on the fibers of the pulp as economically as possible.

A means for carrying out the process is shown in the accompanying drawing which is a section through a mold containing iron turnings and magnesium carbonate.

According to the present invention wire-network, iron turnings or such meltable objects are placed in the mold employed for casting the working parts in question, so that the molten metal when poured into the mold becomes agitated, by which action a flaw-formation is caused, which makes the metal-mass porous. This flaw-formation can be increased by mixing the molten metal with calcic or magnesium-carbonate or other gasgiving substances, which by the forming of gas produces flaws in the material and make it porous.

Preferably the method is so carried out by placing the iron turnings or the wire-network in the molds at a suitable distance from each other, after which the molten metal is poured into the molds. When it comes in contact with the objects put into the mold, the temperature of which is lower than the molten metal, the latter becomes agitated, causing a flaw-formation in the material and making the latter porous. If

gasgiving substances are to be used, they are placed upon the iron turnings, wire-networks or the like.

It is obvious, that material made in the above manner possesses the durability of steel, and that, when used in breaking engines, wood-pulp mills and similar apparatus intended for grinding wood-pulp, there will be no danger of damaging the fibers of the wood-pulp owing to the porous structure.

Having now particularly described and ascertained the nature of our said invention and in what manner the same is to be performed, we declare that what we claim is:

1. A method of forming working parts for apparatus intended for grinding wood-pulp, consisting in placing a gas producing substance in the mold and then pouring the molten metal into the mold, whereby there will be an agitation producing flaws in the material as it hardens, thereby rendering it porous.

2. A method of forming working parts for apparatus intended for grinding wood-pulp, consisting in placing meltable objects spaced from one another in the mold, placing a gas producing substance within said mold and upon said objects, and then pouring the molten metal into the mold, whereby there will be an agitation and formation of gas producing flaws in the material, thereby rendering it porous.

In testimony whereof we have signed our names to this specification in the presence of two subscribing witnesses.

CARL FREDRIK SÖDERVALL.

Witnesses:

VALFRID HANSON.

C. A. HANSON.

HENNING HELIN.

Witnesses:

BIRGER DAHL,

EDWIN WETTERLING.